

## UNITED STATES PATENT OFFICE.

ROBERT R. APPLEGATE AND JOHN B. AUSTIN, OF CLEVELAND, OHIO, ASSIGNORS TO RAIL WELDING AND BONDING COMPANY, OF CLEVELAND, OHIO, A CORPORATION OF DELAWARE.

## METHOD AND MEANS OF UNITING COPPER TO STEEL.

No Drawing.

Application filed March 13, 1922. Serial No. 543,486.

To all whom it may concern:

Be it known that we, ROBERT R. APPLEGATE and JOHN B. AUSTIN, citizens of the United States, and residents of Cleveland, in the county of Cuyahoga and State of Ohio, have invented a certain new and useful Improvement in Methods and Means of Uniting Copper to Steel, of which the following is a specification.

10 This invention relates to the art of arc welding and is especially concerned with a method and means of uniting copper bonds to steel rails.

One object of the invention is to provide a 15 new and improved method of introducing degasifying substances continuously and in predetermined quantities into the molten metal forming the weld metal in a metallic joint.

20 Another object is to provide a welding or filler rod or electrode for use in the process of joining copper bonds to steel rails, having a suitable content of degasifying substance more or less uniformly distributed therein.

25 Another object is to provide a copper filler rod or electrode containing silicon for use in the process of uniting copper bonds to steel rails.

Other objects will appear and be pointed 30 out hereinafter.

Heretofore, so far as we are aware, difficulty has been experienced in uniting copper to copper or copper to steel in a manner to obtain a strong mechanical, good electrically conductive junction. A primary cause of such unsatisfactory joints is the presence of gases either combined or occluded, or both, in the molten copper which are liberated from combination with the

40 molten metal as the metal cools but which remain entrapped therein thus causing porosity. We have discovered that when these gases are suitably removed as such from the molten metal a dense, close grained,

45 metallic structure is obtained which, by reason of its nonporous structure forms a stronger, more highly conductive junction. We have further discovered that highly satisfactory junctions may be obtained if the

50 copper is treated with a degasifying substance thruout the melting thereof and prefer to add the degasifying substance along with each increment of copper melted in the

proportion and amount required for complete degasification of such increment. 55

Such addition of degasifying substance may be accomplished by incorporating in the copper to be melted the substance in a substantially uniformly distributed condition, which is easily possible if such degasifying 60 substances are employed as are readily soluble or capable of more or less uniform distribution in the copper.

Inasmuch as a part of the copper article is usually melted in the process of joining it to a steel or copper article we prefer to employ 65 slightly more degasifying substance in the added copper than is needed for its degasification so that the molten portion of the copper article will be suitably degasified. 70 In a similar manner pure copper melted into the joint may be provided for.

We prefer to employ silicon as a degasifying substance but there are many other more or less suitable substances including 75 aluminum, phosphorus, magnesium, boron and manganese, any one or more of which may be utilized. For the sake of brevity we have used the terms "copper" and "steel" 80 in this specification but we regard copper base alloys and iron, as full equivalents of the copper and steel mentioned above; and accordingly intend the above terms to include these and other equivalent metals.

As a specific illustration of our improved 85 method of uniting copper to steel, we have selected for description its application to the method of attaching electrically conductive copper bonds to steel railways rails, as practised heretofore and disclosed in Letters 90 Patent of the United States 1,183,992, and 1,183,993.

In practising our invention we prefer to follow a part of the process outlined in said 95 patents, but to use copper filler wire containing predetermined amounts of silicon to complete the bond head, instead of ordinary copper as used heretofore.

The silicon should be more or less uniformly distributed thruout the copper so 100 that as the copper melts, each molten part carries with it sufficient silicon for its degasification. When such amounts or proportions of silicon to copper are maintained the gases in each molten part of copper are 105 rendered harmless or removed shortly after

such part is melted, the addition of degasifying substance beginning with the first molten metal, continuing as long as metal is melted and always being present in substantially the required amount for best results.

The silicon content may vary over a relatively small range, preferably between about .22% and .35% by weight. A silicon content of about .25% has given good results. The degasifying substance need not, and preferably should not, be used in such amounts in the copper as to remain in considerable amounts in the finished bond head. 15 When the silicon content is about as stated above only about 0.12% will be found in the solidified metal. We have found that such amounts of silicon are adequate also to degasify portions of the bond head which 20 are ordinarily melted in the process.

Copper containing silicon for use in making bond heads may be conveniently formed into rods or wires, which form also lends itself readily to a variation of the silicon content in the molten metal by wrapping the rods with or around scrap copper.

Bonds attached to rails by this method have been found to be of close grained, substantially nonporous structure and to be many times more firmly attached mechanically to the rail and to have a much higher electrical conductivity than bonds attached by the methods practised heretofore. These notable improvements are due largely, we believe, to our improved method and means of removing substantially all gases as such from the molten bond head metal before solidification thereof.

Although we have described our invention in detail as applied to the attaching of bonds to rails, we do not wish to be limited thereto since broadly our invention is applicable in the uniting of copper to copper or copper to steel where maximum strength and electrical conductivity are desired.

The scope of our invention is defined by what is claimed.

What is claimed is:—

60 1. The method of joining a copper bond to a steel rail which comprises forming a

suitable mold cavity about a portion of the copper of a bond to retain molten metal in contact with the rail and melting into the mold cavity copper having incorporated 55 therein a substantial amount and up to about .35% by weight of silicon to join the bond to the rail.

2. The method of joining a copper bond to a steel rail which comprises forming a 60 suitable mold cavity about a portion of the copper of a bond to retain molten metal in contact with the rail, melting into the mold cavity a part of the bond and additional copper containing approximately 65 .25% by weight of silicon substantially uniformly distributed therein to join the bond to the rail.

3. The method of joining a copper bond to a steel rail which comprises forming a 70 suitable mold cavity about a portion of the copper of a bond to retain molten metal in contact with the rail, melting into the mold cavity by means of an electric arc a part of the bond and additional copper having incorporated therein a substantial amount and up to about .35% by weight of silicon to complete the bond head and joining the bond to the rail.

4. As a new article of manufacture, a 80 copper welding rod containing silicon in a substantial amount and up to about .35% substantially uniformly distributed therein.

5. As a new article of manufacture, copper for use in joining copper to steel containing silicon from about .22% to .35%. 85

6. As a new article of manufacture, copper wire for use in joining copper to steel containing about .25% of silicon by weight.

7. As a new article of manufacture, an 90 alloy welding rod consisting predominantly of copper and having silicon distributed substantially uniformly therein in a substantial amount and up to about .35%.

8. As a new article of manufacture, copper for use in joining copper to steel containing silicon in a substantial amount and up to about .35%. 95

In testimony whereof, we hereunto affix our signatures.

ROBERT R. APPLEGATE.  
JOHN B. AUSTIN.